

## UNITED STATES PATENT OFFICE

LEON LILIENFELD, OF VIENNA, AUSTRIA

## PROCESS FOR IMPROVING COTTON

No Drawing. Application filed February 3, 1927, Serial No. 165,749, and in Austria May 23, 1923.

There are known processes of treating vegetable fibrous materials, such as cotton fabric and the like, with alkali and carbon bisulphide, partly in order to convert these materials into a parchment-like product, partly to provide them with a durable dressing. These processes consist in treating the fibrous materials, particularly fabrics, with strong alkali solution and then subjecting them to the action of carbon bisulphide in vapour form, or in treating the material first with concentrated alkali solution, then with carbon-bisulphide and finally mercerizing under tension.

According to my invention very valuable properties are imparted to cotton in hank or fabric form when, without previously converting it into alkali-cellulose, it is treated simultaneously with alkali solution and carbon bisulphide, undiluted or diluted with suitable diluents (for example, benzene, chloroform, petrol, petroleum ether, ligroin, carbon tetrachloride or the like). This may be done either by impregnating the cotton or the material consisting of or containing cotton with diluted or undiluted carbon bisulphide and then similarly treating with alkali solution or by subjecting the cotton material to the action of alkali solution to which carbon bisulphide is added before or after the introduction of the cotton.

According to the particular nature of the cotton material and the duration of the action of the carbon bisulphide in presence of alkali solution, there are obtained according to the present process either highly-translucent effects with a very silky lustre, or a more or less stiffening finishing or both. Wool-like appearance and feel may also be given to the material treated according to the process,

The cotton may be treated according to the invention in the form of fabric, of yarns, in hanks or in the form of cops or warps.

The cotton or the material consisting of or containing cotton, may be treated by the present process raw or after preliminary treatment (for example boiled, wetted or not wetted, unbleached or bleached with oxidizing or reducing bleaching agents, mercerized or not mercerized).

It may also be treated previously with a hydrolyzing or gelatinizing agent, for example a strong mineral acid, such as sulphuric acid of 49-60° Baumé specific gravity or phosphoric acid of 55-57° Baumé or higher specific gravity, or hydrochloric acid of 24° Baumé specific gravity, or nitric acid of 43-46° Baumé or higher specific gravity, or hot solution of zinc chloride of 60° Baumé specific gravity or an ammoniacal solution of cupric oxide of considerable concentration.

By reserving certain portions in accordance with known methods (for example by the application of substances adapted for this purpose, such as albumin, gum, acids and the like) pattern effects may be obtained by the present process.

Mixed goods, that is to say, goods composed of vegetable and animal fibres, may also be subjected to the present process.

By suitable selection of the operating conditions there may be obtained in accordance with the present process silky effects surpassing those obtained by the usual mercerizing methods, as well as wool-like or springy effects.

To obtain the silky lustre, stretching of the goods is essential. It is immaterial whether the tension is applied before or after the treatment with alkali solution in presence of carbon bisulphide. When the stretching of the goods is omitted the silky lustre effects disappear and the goods assume a springy condition and resemble wool to a very marked degree.

The following examples illustrate the invention:

1. Bleached or unbleached mercerized or unmercerized cotton fabric is treated under tension with carbon bisulphide undiluted or diluted with benzene (for example 1-5 parts of benzene to 1 part of carbon bisulphide) for some seconds up to a quarter of an hour. Then, where desired after squeezing out the excess carbon bisulphide, the fabric is treated with caustic soda solution of 14-20 per cent strength for some minutes up to several hours.

2. Cotton fabric under tension is introduced into a mixture of caustic soda solution of 10-18 per cent strength with 0.2-3.0 per cent

cent of carbon bisulphide and treated with this mixture for some minutes up to several hours.

3. The mode of operation is as in the foregoing examples, except that before being subjected to the present process the fabric is previously treated with a strong sulphuric acid. If a sulphuric acid of 49-50° Baumé specific gravity is used for this purpose, the treatment therewith, at room temperature, may be continued for a few seconds up to some minutes or even longer. If a stronger sulphuric acid is used, for example one of 52-54° Baumé specific gravity, the treatment is to occupy only a few seconds, if the sulphuric acid is of room temperature. If the sulphuric acid is cooled to 0° C. or lower, the treatment may be longer.

The treatment with sulphuric acid may be preceded by a mercerizing of the fabric, for example with caustic soda solution of 10 per cent strength at low temperatures or with a strong caustic soda solution, for example of 18-40 per cent strength at room temperature.

23. In order to bring about the production of the wool-like effects or wooly appearance of the goods treated, it only becomes necessary to omit what was said above to be essential to the production of the silky effects, namely 30 the treatment of the goods under tension or in the stretched condition. Therefore, if the wool-like appearance or springy condition of the goods treated is desired, it may be produced simply by omitting the stretching 35 or tension referred to in the above specific examples.

The cotton fabric treated in accordance with the present process may, of course, be washed or acidified and washed and dried in the usual way. It may also be dried or 40 steamed before washing.

All the secondary operations usual in mercerizing or proposed therefor may be applied to the present process, for example lustering, 45 printing, etc.

The finished fabrics may, if desired, be calendered, schreinered, beatled or the like.

The term "cotton" in the following claims 50 comprises cotton in the form of pure cotton or mixed fabrics, of yarns for example in hanks or cops or warps.

The expression "mercerizing agent" in the following claims comprises alkali lye or strong mineral acids.

55. This application is in part a continuation of my application Serial No. 712,473, filed May 10, 1924.

I claim:

60. 1. The process of imparting wool-like effects to cotton by treatment with caustic alkali and carbon bisulphide, which comprises treating cotton in a substantially unstretched or free from tension condition, 65 without previous conversion into caustic

alkali cellulose, simultaneously with caustic alkali solution and carbon bisulphide.

2. The process of imparting wool-like effects to cotton by treating with caustic alkali and carbon bisulphide which comprises treating cotton in a substantially unstretched or free from tension condition first with carbon bisulphide and then with caustic alkali solution. 70

3. The process of imparting wool-like effects to cotton by treating with caustic alkali and carbon bisulphide which comprises reacting upon cotton in a substantially unstretched condition with a mixture of caustic alkali solution and carbon bisulphide. 75

4. The process of producing wool-like effects in cotton goods which comprises subjecting cotton goods to the simultaneous action of carbon bisulphide and a hydroxide of an alkali metal while maintaining the cotton goods during such action in a substantially unstretched condition or in a state substantially free from tension. 80

5. The process of imparting wool-like effects to cotton by treatment with alkali and carbon disulphide which comprises reacting simultaneously on cotton in a substantially unstretched or free from tension condition with caustic alkali and carbon disulphide. 85

6. The process of imparting wool-like effects to cotton by treatment with caustic alkali and carbon bisulphide which comprises treating cotton in a substantially unstretched, or free from tension condition, and while substantially free from previously formed alkali cellulose, first with carbon bisulphide and then with aqueous caustic alkali solution. 90

7. The process of imparting wool-like effects to cotton by treatment with caustic alkali and carbon bisulphide which comprises subjecting the cotton in a substantially unstretched or free from tension condition, and while substantially free from previously formed alkali cellulose, to the action of a mixture of carbon bisulphide and aqueous caustic alkali. 100

In testimony whereof I affix my signature.  
LEON LILIENFELD.

115

120

125

130